

# United States Patent

Tammela et al.

[15] 3,649,341

[45] Mar. 14, 1972

[54] **METHOD FOR MANUFACTURING  
PARTIALLY ACYLATED  
REGENERATED CELLULOSE FOIL OR  
FIBER**

- [72] Inventors: **Viljo Tammela, Helsinki; Olli Turunen, Porvoo; both of Finland**
- [73] Assignee: **Neste Oy, Helsinki, Finland**
- [22] Filed: **Nov. 14, 1968**
- [21] Appl. No.: **775,952**

[30] **Foreign Application Priority Data**

- Nov. 17, 1967 Finland.....3106/67
- [52] U.S. Cl.....117/118, 8/121, 117/60,  
117/144
- [51] Int. Cl.....B44d 51/2, D06m 13/20
- [58] Field of Search .....8/120, 121; 117/60, 144.5,  
117/144, 118

[56] **References Cited**

UNITED STATES PATENTS

- 2,036,947 4/1936 McKee et al.....8/121 UX

|           |         |                    |       |
|-----------|---------|--------------------|-------|
| 2,772,944 | 12/1956 | Allewell.....      | 8/121 |
| 2,780,511 | 2/1957  | Takagi.....        | 8/121 |
| 3,215,490 | 11/1965 | Fraizy et al. .... | 8/121 |

**FOREIGN PATENTS OR APPLICATIONS**

|         |        |                    |       |
|---------|--------|--------------------|-------|
| 353,978 | 8/1931 | Great Britain..... | 8/121 |
| 448,063 | 6/1936 | Great Britain..... | 8/121 |
| 750,702 | 6/1956 | Great Britain..... | 8/121 |
| 930,208 | 7/1963 | Great Britain..... | 8/121 |

*Primary Examiner*—William D. Martin

*Assistant Examiner*—M. R. Lusignan

*Attorney*—Richards & Geier

[57]

**ABSTRACT**

Partly acetylated regenerated cellulose films or fibers are manufactured by first swelling them in a concentrated and water-free acetic acid solution of an alkali metal acetate at a temperature ranging between 50° and 140°. Immediately thereafter and without drying the swelled films or fibers are esterified by an acetic acid anhydride solution containing alkali metal acetate at a temperature ranging between 100° and 170° C.

**1 Claims, No Drawings**

**METHOD FOR MANUFACTURING PARTIALLY  
ACYLATED REGENERATED CELLULOSE FOIL OR  
FIBER**

The present invention concerns a method for manufacturing partially acylated cellulose foil or fiber in which the foil or fiber which is to be esterified is at first swollen at elevated temperature and subsequently esterified, whereupon the product is washed and dried.

Since regenerated cellulose presents drawbacks as low wet strength and brown discoloration at high temperatures, methods have been developed in which the properties of regenerated cellulose foil or fiber are improved by means of partial acylation. By such methods the objectionable characteristics of regenerated cellulose foil or fiber can indeed be eliminated because partially acylated regenerated cellulose foil or fiber has good heat resistance and high wet strength. In the acylating methods of previous art initial treatment of the regenerated cellulose foil or fiber has been accomplished by first swelling the foil or fiber in aqueous solutions of salts, after which step it has been necessary to dry the swollen foil or fiber prior to esterification and only after this has the acylating process been performed with acid anhydrides. If acid esterification catalysts have been used as components in the acid anhydride solution, it has furthermore been necessary prior to esterification to remove by washing the salts absorbed by the foil and fibers during the swelling process. As a consequence of the circumstances mentioned, the acylating methods employed up to date have in fact been slow and complicated. In addition, partial depolymerization and discoloration of the cellulose may occur.

The object of the present invention is to afford a method for acylating regenerated cellulose foil or fiber which is superior to previous methods in speed and simplicity. The invention is accordingly mainly characterized in that swelling of the foil or fiber is accomplished in a substantially water-free aliphatic carboxylic acid solution containing salt of an alkali metal and an aliphatic carboxylic acid and that the product thus obtained is immediately esterified in a manner previously known in itself in a solution of the anhydride of a low-molecular carboxylic acid which contains salt of an alkali metal and an aliphatic carboxylic acid. Since it is not necessary in a method according to the invention to dry the swollen foil or fiber because the foil or fiber is swollen in a substantially water-free swelling solution, nor to wash it because esterification may be accomplished immediately after swelling without causing any damage to the foil or fiber, it follows that a method according to the invention surpasses any previous methods in the speed and simplicity with which it can be carried out.

It has been found that alkali metal salts of low-molecular aliphatic carboxylic acids, solved in aliphatic carboxylic acids, are most effective for use as cellulose-swelling agents in the method for manufacturing partially acylated regenerated cellulose concerned here. Alkali metal acetates solved in acetic acid have been found to be the most efficient ones among them.

The composition of the acid anhydride solutions used in the method may vary considerably. It is possible to use for acylating agent merely the anhydride of some low-molecular carboxylic acid or a mixture of these. With increasing molecular size of the anhydrides increasingly soft products are obtained, e.g., compared to the use of acetic acid anhydride alone.

For use as reaction accelerators in the esterifying solution the same salts are most effective as are used for bloating agents in the pretreatment.

It is possible to use as raw material e.g., unsoftened regenerated cellulose foil or fiber.

Pretreatment is accomplished by immersing the regenerated cellulose foil or fiber into a swelling bath at elevated temperature, e.g., at 50°-140° C.

The pretreated product thus obtained is immediately immersed, without intervening drying, into the esterifying solution at elevated temperature, e.g., at 100°-170° C.

After completed esterification the acylated foil is washed with acetic acid and with water. Fiber may also be washed

with water alone, whereby the luster characteristic of the fibers can be dulled.

The foils or fibers may be bleached upon completed washing if necessary.

If a more flexible product is desired, the partially acylated product may also be immersed into a solution containing a softener prior to drying.

Drying is accomplished by the usual method employed for regenerated cellulose.

By a method according to the invention partially acylated regenerated cellulose foil or fiber with good heat resistance and possessing wet strength is obtained.

The dry tensile strengths of the foils were determined according to the ASTM D 1708-59 method. The determination of wet tensile strength differed from the said method in that the test specimens were kept immersed in water at room temperature for 20 hours prior to the tensile test. The average dry and wet strengths of the original regenerated cellulose foils were 1,300 and 200 kp/cm.<sup>2</sup>. The determinations of heat resistance were carried out according to the ASTM D 1637-61 method, stating as the heat resistance of the foil the temperature at which the elongation of the specimen was 2 percent of its original length. The heat resistance of the regenerated cellulose foil, according to the ASTM D 1637-61 method, was >200° C.

The brown discoloration of the foils was studied by keeping the samples for 1 hour at 210° C. and, subsequently, determining their transparency with a spectrophotometer according to the ASTM D 1746-62 method. The transparencies were stated in percent at the wavelengths of 400 and 550 m $\mu$ . Prior to the heat treatment, the transparencies of the original as well as the partially regenerated cellulose foil amounted to 84-85 percent at 400 m $\mu$  and to 87-88 percent at 550 m $\mu$ . The transparency of the original regenerated cellulose foil after heating for 1 hour at 200° C. was 67-70 percent at 550 m $\mu$  and 40-42 percent at 400 m $\mu$ .

The method according to the invention is illustrated by a few examples in the following.

**EXAMPLE 1**

Regenerated cellulose foil (thickness 25 $\mu$ ) was immersed for swelling for a period of 1 minute into a solution of 45 parts by weight potassium acetate and 55 parts by weight acetic acid at 98° C. Immediately after, the foil was immersed for 1 minute into the boiling esterifying solution, which had the following composition:

|    |                   |                    |
|----|-------------------|--------------------|
| 50 | Acetic anhydride  | 98 parts by weight |
|    | Potassium acetate | 2 parts by weight  |

Acetylation was followed by washing for 30 seconds in acetic acid at room temperature, whereupon the foil was furthermore washed with water, and dried. The clear foil which was obtained had the following properties:

|    |                 |          |
|----|-----------------|----------|
| 60 | Thickness       | 37 $\mu$ |
|    | Acetyl content  | 24%      |
|    | Heat resistance | >200° C. |

Transparency after the discoloration test, at 400 m $\mu$  74-75 percent, at 550 m $\mu$  84-85 percent

|    |                      |                         |
|----|----------------------|-------------------------|
| 65 | Wet tensile strength | 362 kp/cm. <sup>2</sup> |
|    | Dry tensile strength | 824 kp/cm. <sup>2</sup> |

**EXAMPLE 2**

The test was performed as in Example 1, but the esterifying solution had a different composition, which was:

|    |                   |                    |
|----|-------------------|--------------------|
| 70 | Acetic anhydride  | 92 parts by weight |
|    | Potassium acetate | 5 parts by weight  |
|    | Acetic acid       | 3 parts by weight  |

75 The end product had the following properties:

|                 |          |
|-----------------|----------|
| Thickness       | 37 $\mu$ |
| Acetyl content  | 23%      |
| Heat resistance | >200° C. |

Transparency after the discoloration test, at 400 m $\mu$  73-74 percent, at 550 m $\mu$  84-85 percent

|                      |                         |
|----------------------|-------------------------|
| Wet tensile strength | 338 kp/cm. <sup>2</sup> |
| Dry tensile strength | 815 kp/cm. <sup>2</sup> |

### EXAMPLE 3

The procedure applied in the test differed from that in Example 1 only in respect of the esterifying solution, which was:

|                   |                    |
|-------------------|--------------------|
| Acetic anhydride  | 85 parts by weight |
| Potassium acetate | 5 parts by weight  |
| Acetic acid       | 10 parts by weight |

The foil which was obtained had the following properties:

|                 |          |
|-----------------|----------|
| Thickness       | 33 $\mu$ |
| Acetyl content  | 16.6%    |
| Heat resistance | >200° C. |

Transparency after the discoloration test, at 400 m $\mu$  60-70 percent, at 550 m $\mu$  80-82 percent

|                      |                         |
|----------------------|-------------------------|
| Wet tensile strength | 304 kp/cm. <sup>2</sup> |
| Dry tensile strength | 956 kp/cm. <sup>2</sup> |

### EXAMPLE 4

The test was performed as in Example 1, but a regenerated cellulose fiber bundle was used instead of regenerated cellulose foil. In addition, the acetylating solution had a composition differing from that mentioned above, and it was:

|                   |                    |
|-------------------|--------------------|
| Acetic anhydride  | 92 parts by weight |
| Potassium acetate | 4 parts by weight  |
| Acetic acid       | 4 parts by weight  |

After esterifying for 90 seconds, the acetyl content of the regenerated cellulose fiber was found to be 24.4 percent.

### EXAMPLE 5

The test was performed in Example 1, but the composition of the esterifying solution was different; it was:

|                   |                    |
|-------------------|--------------------|
| Acetic anhydride  | 95 parts by weight |
| Potassium acetate | 5 parts by weight  |

After acetylation for 1 minute and after the subsequent washings, the foils had the following properties:

|                 |          |
|-----------------|----------|
| Thickness       | 40 $\mu$ |
| Acetyl content  | 35%      |
| Heat resistance | 190° C.  |

Transparency after the discoloration test, at 400 m $\mu$  76-77 percent, at 550 m $\mu$  83-86 percent

|                      |                         |
|----------------------|-------------------------|
| Wet tensile strength | 402 kp/cm. <sup>2</sup> |
| Dry tensile strength | 760 kp/cm. <sup>2</sup> |

### EXAMPLE 6

The test was performed as in Example 1, but the composition of the esterifying solution was different from that mentioned above; it was:

|                   |                    |
|-------------------|--------------------|
| Acetic anhydride  | 48 parts by weight |
| Butyric anhydride | 48 parts by weight |
| Potassium acetate | 4 parts by weight  |

After acetylation for 2 minutes and subsequent washings, the foils had the following properties:

|           |          |
|-----------|----------|
| Thickness | 45 $\mu$ |
|-----------|----------|

|                 |         |
|-----------------|---------|
| Acetyl content  | 28.4 %  |
| Butyryl content | 5.2%    |
| Heat resistance | 200° C. |

Transparency after the discoloration test, at 400 m $\mu$  76 percent, at 550 m $\mu$  86 percent

|                      |                         |
|----------------------|-------------------------|
| Wet tensile strength | 350 kp/cm. <sup>2</sup> |
| Dry tensile strength | 710 kp/cm. <sup>2</sup> |

10 The dry elongation was found to be 15 percent, whereas the dry elongation of merely acetylated foils is in the order of 10-12 percent; the addition of butyryl content thus exerts a plasticizing effect on the foils.

### EXAMPLE 7

The test was performed as in Example 1, but commercial regenerated cellulose foil (plasticizer content, about 10 percent) was used instead of isotropic foil. The esterifying solution had the following composition:

|                   |                    |
|-------------------|--------------------|
| Acetic anhydride  | 96 parts by weight |
| Potassium acetate | 4 parts by weight  |

25 After acetylation for 1 minute and subsequent washings, the foils had the following properties:

|                 |          |
|-----------------|----------|
| Thickness       | 28 $\mu$ |
| Acetyl content  | 30%      |
| Heat resistance | >200° C. |

30 Transparency after the discoloration test:

|                |     |
|----------------|-----|
| at 400 m $\mu$ | 76% |
| at 550 m $\mu$ | 87% |

(Original, 21%)

(Original, 63%)

35 Wet tensile strength in the machine direction

|                         |
|-------------------------|
| 435 kp/cm. <sup>2</sup> |
|-------------------------|

(Original, 225 kp/cm.<sup>2</sup>)

40 Wet tensile strength across the machine direction

|                         |
|-------------------------|
| 250 kp/cm. <sup>2</sup> |
|-------------------------|

(Original, 140 kp/cm.<sup>2</sup>)

Dry tensile strength in the machine direction

|                          |
|--------------------------|
| 1010 kp/cm. <sup>2</sup> |
|--------------------------|

(Original, 1120 kp/cm.<sup>2</sup>)

Dry tensile strength across the machine direction

|                         |
|-------------------------|
| 615 kp/cm. <sup>2</sup> |
|-------------------------|

(Original, 500 kp/cm.<sup>2</sup>)

50 Comparison of the acetyl contents of the foils obtained in Examples 2 and 3 reveals that the acetic acid present in the esterifying solution retards the reaction rate. This detriment can be avoided in a continuous process either by removing the acetic acid from the esterifying solution or by adding to it salt used to accelerate the reaction, whereby the acylating rate can be maintained virtually constant.

It is seen from the examples presented that in a method according to the invention the acetylating process takes less than 5 minutes, exclusive of potential bleaching, washing with water and drying.

The wet strength of the partially esterified (acetyl content, 30-35 percent) regenerated cellulose foil (400 kp/cm.<sup>2</sup>) is markedly better than that of the merely regenerated cellulose foil (200 kp/cm.<sup>2</sup>) and nearly equals that of cellulose acetate foils (450 kp/cm.<sup>2</sup>). The heat resistance of partially acetylated regenerated cellulose foil is >200° C. if the acetyl content is <33 percent. Such partially esterified cellulose foil is not soluble in a cellulose solvent such as Cadoxene solution nor in cellulose acetate solvents such as acetone, 2-methoxy ethanol acetic acid or chloroform.

We claim:

1. The method for manufacturing partly acetylated regenerated cellulose film or fibers, which comprises swelling

the film or fibers in a substantially water-free acetic acid solution of an alkali metal acetate at a temperature of 50°-140° C. and immediately thereafter esterifying them without drying by an acetic acid anhydride solution containing alkali metal acetate at a temperature of 100°-170° C. and then washing 5 and drying them.

\* \* \* \* \*

10

15

20

25

30

35

40

45

50

55

60

65

70

75